

(No Model.)

C. L. COFFIN.

PROCESS OF ELECTRIC WELDING.

No. 396,270.

Patented Jan. 15, 1889.



Fig. 2



Fig. 1

Witnesses.

Geo. H. Lothrop.

Adelaide A. Anderson.

Inventor  
Charles L. Coffin.

# UNITED STATES PATENT OFFICE.

CHARLES L. COFFIN, OF DETROIT, MICHIGAN.

## PROCESS OF ELECTRIC WELDING.

SPECIFICATION forming part of Letters Patent No. 396,270, dated January 15, 1889.

Application filed June 19, 1888. Serial No. 277,513. (No model.)

*To all whom it may concern:*

Be it known that I, CHARLES L. COFFIN, of Detroit, in the county of Wayne and State of Michigan, have invented a new and useful 5 Improvement in Electric Welding, of which the following is a specification.

My invention consists in an improved process of electric welding, hereinafter fully described and claimed.

10 The process consists in forming the voltaic arc in such manner that it shall extend outside of a straight line joining the ends of a positive and negative conductor, and then drawing the conductors while the current is 15 passing along the joints to be welded, whereby the joint is submitted to the action of the voltaic arc; and, as an addition to this process, my invention further consists in feeding to the joints to be welded and within the influence 20 of the voltaic arc a strip of metal, which is fused by the arc and deposited on or in the joint, whereby the welded joint is re-enforced.

The apparatus by which my process may be carried out may be varied in form or construction, it only being necessary that the arc 25 when formed shall spring beyond the ends of the carbons, which may be done either by the position of the carbons or by deflecting the arc magnetically in a well-known manner.

30 A mechanism which may be used to practice my process is illustrated in the accompanying drawings, in which—

Figures 1 and 2 are front elevations, being exactly alike except that Fig. 2 has added a 35 guide for feeding the re-enforcing piece of metal.

B represents a carbon-holder, and A represents a box on said holder, containing mechanism for feeding the carbons as they are 40 worn away, which is not shown, as it forms no part of the invention designed to be hereby secured.

C represent two carbon pencils secured in holder B at an angle with each other, 45 whereby the voltaic arc L is sprung outward from the straight line joining the point of the carbons, as shown in the figures, so that this are may be brought into contact with the joint to be welded without touching the joint 50 with the carbon.

F represents an insulated handle for the carbon-holder B, by which it may be operated by an attendant.

G H represent binding-posts through which the poles of the generator may be connected 55 with carbons C C.

E represent insulated rollers, which may be used to support the holder B and permit it to be drawn along the joints, the rollers S resting either on the sheets of metal to be 60 welded or on table carrying the work. These may be used or not, as willed.

In Fig. 2, I represents a guide, consisting of a hollow pipe secured to the carbon-holder B, and D represents a wire or strip of metal, 65 which passes through the carbon-holder and through said guide I, so that its end passes between the points of the carbons C C without touching either of them. The wire D should preferably be insulated from the carbon-holder B, so that it cannot possibly short-circuit the carbons. It is evident that when 70 the points of the carbon are placed over the joints to be welded the end of the wire D will lie upon the joint, and that it will be fused by the voltaic arc at the same time the joint 75 is fused, whereby the fused portion of the wire D will be laid along the joint, thereby re-enforcing the welding.

I am aware that prior patents have described the process of electric welding in which the voltaic arc has been sprung between the metal to be welded as one pole and a movable conductor as the other pole, and do not claim any such process herein. 80

85 What I claim as my invention, and desire to secure by Letters Patent, is—

1. The herein-described process of electric welding, consisting in forming a voltaic arc between two conductors extending outward 90 from said conductors and submitting the joint to be welded to the action of said arc.

2. The herein-described process of electric welding, consisting in forming a voltaic arc between two conductors extending beyond 95 the points thereof, feeding a strip of metal into the arc between the conductors, and submitting the joints to be welded and said strip of metal simultaneously to the action of said arc.

CHARLES L. COFFIN.

Witnesses:

ADELAIDE A. ANDERSON,  
GEO. H. LOTHROP,